

# UNITED STATES PATENT OFFICE.

HARRY S. MORK, OF BROOKLINE, MASSACHUSETTS, ASSIGNOR TO AMERICAN  
LA FRANCE FIRE ENGINE COMPANY, INC., OF ELMIRA, NEW YORK, A COR-  
PORATION OF NEW YORK.

## FIRE-EXTINGUISHER COMPOSITION.

1,246,640.

Specification of Letters Patent.

Patented Nov. 13, 1917.

No Drawing.

Application filed February 26, 1917. Serial No. 151,099.

To all whom it may concern:

Be it known that I, HARRY S. MORK, a citizen of the United States, and resident of Brookline, county of Norfolk, State of 5 Massachusetts, have invented a certain new and useful Fire-Extinguisher Composition, of which the following is a specification.

My invention relates in general to fire extinguishing compounds or compositions of 10 the type embodying substances for the production of a relatively heavy blanket of gas or vapor to smother the fire, while at the same time possessing in its normal state, a permanence and so-called nonfreezing character. Carbon-tetrachlorid has already been proposed and employed as a principal component of such compositions, and other substances have been added to the carbon-tetrachlorid to lower its freezing point, to 15 retard the dispersion of the gas or vapor which is produced when the composition is employed for extinguishing the fire, and to reduce the corrosive action of the liquid on the metal of the container in which it is 20 stored for use.

The objects of my invention are to provide an efficient fire extinguishing composition of low freezing point.

The fire extinguishing composition according to my invention, comprises as its 30 essential ingredients, carbon-tetrachlorid, chloroform, and an aromatic ester, or a mixture of aromatic esters of relatively high boiling point, particularly a phenyl ester, 35 or esters, as for example, triphenyl-phosphate and phenyl salicylate (salol). I prefer to use triphenyl-phosphate, which is a crystalline solid, as one of the esters, on account of its non-inflammable properties, and 40 I furthermore prefer a mixture of triphenyl-phosphate and phenyl salicylate because proper mixtures of these two esters are liquid even at ordinary temperatures. The proportions of these ingredients may be varied, but in any case, carbon-tetrachlorid 45 constitutes the major portion of the composition. The addition of chloroform to carbon-tetrachlorid has a very marked effect in depressing the freezing point, whereas the 50 other two ingredients, triphenyl-phosphate and phenyl salicylate, act in the capacity of forming deposits or coatings upon the burning material. The composition as a whole constitutes a fire extinguishing me-

dium of high efficiency, which can be stored 55 for a long period of time in any of the usual forms of containers, without exhibiting any serious corrosive effect on the metal of the container (usually brass), and it will stand a temperature of minus 50° F. or lower, 60 without freezing. It is clean and free from disagreeable odor.

As an example of a composition which I have found by experiment to have all the good qualities above enumerated, I may refer to the following: carbon-tetrachlorid 65 95%, and chloroform 5% by volume, having for each 100 cubic centimeters of this mixture an addition of 2½ grams of a mixture made up of equal parts of triphenyl-phosphate and phenyl salicylate.

The above composition gives a freezing point close to minus 50° F. and has been found by actual test to cause substantially 75 no corrosion of a brass container, after several weeks exposure at approximately 80° F., and to act as an efficient extinguishing medium. Increased proportions of chloroform, further reduce the freezing point, but increased percentage of triphenyl phosphate 80 and salol have the opposite effect on the composition and require further proportions of chloroform to maintain the desired low freezing point.

It is not essential that both the triphenyl-phosphate and the phenyl salicylate be employed together, although I prefer the composition approximately as above given. I may, for example, add 5 grams triphenyl-phosphate in 100 c. c. of a mixture made up 85 of 95% carbon-tetrachlorid and 5% chloroform, by volume, but this composition would be inferior to the one above given, inasmuch as its freezing point is only about minus 40° F. The same quantity of triphenyl-phosphate in 92½% carbon-tetrachlorid and 7½% chloroform, by volume, would give approximately minus 52° F. as the freezing point, and by varying the carbon-tetrachlorid and chloroform to 90% of the former and 10% 95 of the latter, the freezing point would be in the neighborhood of minus 62° F. The same general results are obtained by similar change in proportions where phenyl salicylate is used alone in place of the triphenyl-phosphate, although increased proportions 10 of the chloroform appear to have a more marked effect in depressing the freezing

- point where phenyl salicylate is employed alone in this way. Obviously, where both of these high boiling point substances are employed, their relative proportions to each other may be varied. I find, however, that the composition of 95% carbon-tetrachlorid and 5% chloroform, containing, for each 100 c. c.  $2\frac{1}{2}$  grams made up of equal parts of triphenyl-phosphate and phenyl salicylate, gives an especially advantageous freezing point with good economy of chloroform, while at the same time offering all the advantages enumerated above for this composition.
- 15 I claim:—
1. A fire extinguishing composition comprising carbon-tetrachlorid, a freezing point lowering component, and an aromatic ester.
  2. A fire extinguishing composition comprising carbon-tetrachlorid, chloroform, and an aromatic ester.
  3. A fire extinguishing composition comprising carbon-tetrachlorid, a freezing point lowering component, and a phenyl ester.
  4. A fire extinguishing composition comprising carbon-tetrachlorid, chloroform, and a phenyl ester.
  5. A fire extinguishing composition comprising carbon-tetrachlorid, a freezing point

lowering component, and a mixture of aromatic esters. 30

6. A fire extinguishing composition comprising carbon-tetrachlorid, chloroform, and a mixture of aromatic esters.

7. A fire extinguishing composition comprising carbon-tetrachlorid, a freezing point lowering component, and a mixture of phenyl esters. 35

8. A fire extinguishing composition comprising carbon-tetrachlorid, chloroform, and a mixture of phenyl esters. 40

9. A fire extinguishing composition containing carbon-tetrachlorid, chloroform and triphenyl-phosphate.

10. A fire extinguishing composition containing carbon-tetrachlorid, chloroform and phenyl salicylate. 45

11. A fire extinguishing composition comprising carbon-tetrachlorid, chloroform, triphenyl-phosphate and phenyl salicylate. 50

12. A fire extinguishing composition comprising substantially a mixture of 95 parts by volume of carbon-tetrachlorid with 5 parts by volume of chloroform, containing for each 100 cubic centimeters of their mixture,  $2\frac{1}{2}$  grams of triphenyl-phosphate and phenyl salicylate in equal parts. 55

HARRY S. MORK.